

# United States Patent [19]

Loriers et al.

[11] 3,779,948

[45] Dec. 18, 1973

[54] VITREOUS COMPOUNDS WITH BISTABLE ELECTRICAL CHARACTERISTICS

[75] Inventors: **Jean Loriers**, Meudon; **Rudolf Heindl**, Fontenay Aux Roses, both of France

[73] Assignee: **Etablissement Public: Agence Nationale de Valorisation de la Recherche Anvar**, Paris, France

[22] Filed: July 28, 1971

[21] Appl. No.: 166,777

## [30] Foreign Application Priority Data

July 31, 1970 France ..... 70.28387

[52] U.S. Cl. .... 252/521, 423/263, 423/464, 423/465, 423/593, 423/594, 423/600,

106/73.1, 106/73.2, 106/73.4, 106/47 R, 338/20

[51] Int. Cl. .... H01c 7/10

[58] Field of Search ..... 252/518, 519, 521; 338/20; 106/39 DV, 39 R, 47 R, 47 Q, 73.1, 73.2, 73.4; 423/464, 465, 593, 594, 600, 263

## [56] References Cited

### UNITED STATES PATENTS

|           |         |                       |           |
|-----------|---------|-----------------------|-----------|
| 3,598,762 | 8/1971  | Futaki et al. ....    | 252/518   |
| 2,862,891 | 12/1958 | Jonker et al. ....    | 252/518 X |
| 3,258,434 | 6/1966  | Mackenzie et al. .... | 252/519   |
| 3,469,729 | 9/1969  | Grekila et al. ....   | 106/47 R  |

3,503,902 3/1970 Shimoda ..... 252/518 X

Primary Examiner—Charles E. Van Horn

Attorney—James and Franklin

## [57] ABSTRACT

A new class of vitreous compounds having bistable electrical characteristics, that is to say, two different states of electric resistance is described.

The new class of vitreous compounds can be represented by the general formula (1):



wherein the letters have the usual meaning of the elements in the Periodic Table with the exception of Ln which designates as a whole a rare earth belonging to the group of lanthanides, such as lanthanum La, or yttrium Y, whereas x, y and z each represent numbers between 0 and 1, which can separately and simultaneously be zero, which are connected by relations of ionic equilibrium, and preferably respond to the inequalities

$$x < 0.15$$

$$y < 0.5$$

and

$$z < 0.3$$

An example of compound having the formula (1) is  $\text{Ca}_2\text{Na}_2\text{Al V}_3\text{O}_{12}$  (II)

10 Claims, 3 Drawing Figures

PATENTED DEC 18 1973

3,779,948

FIG. 1



FIG. 2



FIG. 3



INVENTORS  
JEAN LORIERS  
RUDOLF HEINDL

BY  
James and Franklin  
ATTORNEY

## VITREOUS COMPOUNDS WITH BISTABLE ELECTRICAL CHARACTERISTICS

The object of the invention is a new class of vitreous compounds having bistable electrical characteristics, that is to say, two different states of electric resistance. It also relates to a process for obtaining same and applications thereof.

Vitreous compounds having such characteristics are already known. It is possible, for instance, to mention French patents, 1,445,528 and 1,351,433 as documents illustrating the prior art in this field. Patent 1,445,528 describes binary vitreous compounds. Patent 1,351,433 which is used more particularly as a bibliographical reference in the present description, describes ternary or quaternary vitreous compounds of the type AsTeI, AsTeSe, AsTiSe, VOP, VOPBa, VOPPb or AsBTiO. Such semi-conductive compounds are used in electrical elements where they are combined with an electrical signal source to take advantage of their two states of resistance at least. Said electric elements are used in the technique of switching, in solid state electronic amplifiers and oscillators as well as storage elements, among other things, as the aforesaid French patent explains in detail.

The state of the art with respect to this question can be further illustrated by the following documents: R. and O. HOLZINGER's article headed "Feldabhangige Widerstandsanderung in Glasern" in the German publication "Zeitschrift fur angewandte Physik," vol. 28, No. 4, 1969, pages 196-201, relating to a vitreous compound for electric devices in a conductive and resistant state, which can comprise and adequate mixture of  $\text{B}_2\text{O}_3$ ,  $\text{CaO}$  and  $\text{V}_2\text{O}_5$  oxides.

Swiss patent No. 490,728 (SIEMENS A.G.) relates to a semi-conductive switching device without a junction. A vitreous compound is formed from a mixture of  $\text{V}_2\text{O}_5$  and  $\text{SrCO}_3$ .

United Kingdom Pat. No. 1,168,107 (HITACHI Ltd.) can also be mentioned; it relates to a process for manufacturing a thermistor consisting of a sintered mixture of  $\text{V}_2\text{O}_5$  and a combination of various oxides such as Na, Ca, Al (page 4, example 4), and United States Pat. No. 3,258,434 assigned to (GENERAL ELECTRIC Co) relating to a semi-conductive glass containing  $\text{CaO} \cdot 2\text{B}_2\text{O}_3 \cdot \text{V}_2\text{O}_5 \cdot \text{Fe}_3\text{O}_4 - \text{Al}_2\text{O}_3$  (column 6, example X) as a constituent.

However, the prior art compounds are not satisfactory in all fields of application, and technicians think it desirable to develop vitreous compounds with, notably, improved mechanical and electrical properties.

The object of the present invention is, therefore, vitreous compounds having electrical and mechanical properties very superior to those of similar, known compounds.

The new class of vitreous compounds can be represented by the general formula (1):



wherein the letters have the usual meaning of the elements in the Periodic Table with the exception of Ln which designates as a whole a rare earth belonging to the group of lanthanides, such as lanthanum La, or yttrium Y, whereas  $x$ ,  $y$  and  $z$  each represent numbers between 0 and 1, which can separately and simultaneously be zero, which are connected by relations of ionic equilibrium, and preferably respond to the inequalities

$$\begin{aligned} x &< 0.15 \\ y &< 0.5 \\ \text{and} \\ z &< 0.3 \end{aligned}$$

The chemical composition of the new vitreous compounds appears, at first glance, to be rather complicated. They all, however, have a common basic matrix of formula (II)



(II)

This particular compound corresponding to the formula (I) wherein  $x=y=z=0$ .

The compound of formula (II) has bistable electrical characteristics suited to the requirements of the invention. Its mechanical and electrical properties are superior to those of the known compounds. For example, the difference in resistivities between the conductive and resistant states is at least 10 times as great as that corresponding to the prior compounds.

The other compounds of the invention can be obtained from the basic matrix of formula (II) by the introduction of the rare earth Ln and/or iron Fe or fluorine F.

In certain cases, bistable glasses can also be obtained by combining several compounds corresponding to formula (I), one of which is, for instance, the basic compound of formula (II). The products obtained no longer correspond to formula (I) but they retain bistable electrical characteristics.

A series of examples illustrating said new class of vitreous compounds will be given hereinafter. The common characteristic of these substances is that they have bistable electrical characteristics and that they are vitreous, that is to say, they do not show definite lines in X-ray diagrams (Debye-Scherer diagrams). Said new vitreous compounds are mechanically and chemically very stable, contrary to most of the known compounds which are very friable and very oxidizable glasses containing As, Te, I or the like.

The new vitreous compounds are prepared under critical conditions for precursor products of the chemical elements of formula (I), notably oxides and salts such as carbonates. The mixture of said precursor products in substantially stoichiometric proportions corresponding to formula (I) should be heated at high temperature for a long period of time to obtain vitreous compounds.

The invention therefore also relates to a process for obtaining vitreous compounds corresponding to the aforesaid formula (I) by the intimate contacting of precursor products with the formation of a mixture providing the elements of said compounds in substantially stoichiometric proportions and a thermal treatment, wherein the said mixture is heated for at least 5 hours at a temperature higher than 1,300°C.

Generally speaking, periods of heating from 6 to 12 hours are suitable, at temperatures of 1,300° to 1,400°C, at 1,350°C for example. Melting at insufficiently high temperatures, or for too short periods of time, does not enable vitreous products to be obtained. If the conditions provided for in the invention are not respected, products which crystallize on cooling are finally obtained.

The invention will now be illustrated, while in no way being limited by the following examples:

### EXAMPLE I

Preparation of the compound



(II)

(molecular weight 588.95)

There is prepared an intimate mixture comprising :

 $\text{Al}_2\text{O}_3$  : 0.5 mole or 50.97 g $\text{CaCO}_3$  : 2 moles or 200.18 g $\text{Na}_2\text{CO}_3$  : 1 mole or 106.00 g $\text{V}_2\text{O}_5$  : 1.5 mole or 363.8 g

The total weight of the mixture is therefore 720.95 g.

The mixture is then heated open to the air in a platinum crucible at 650°C for 2 hours, at 750°C for 2 hours and then at 1,350°C for 6 hours.

Chemical analyses effected during heating show that the sodium content does not vary.

The product obtained is a vitreous body corresponding to the aforesaid formula (II) and having two different states of electric resistance.

Electric measurements were carried out to determine the properties of the new product. FIGS. 1 to 3 show the assembly conditions and results obtained.

FIG. 1 is a general diagram of the electric circuit permitting voltage-current characteristics to be obtained.

FIG. 2 is a detailed view showing the assembly of the sample containing product (II).

FIG. 3 is the voltage-current curve obtained.

FIG. 1 shows, diagrammatically, the assembly used. A continuous 300 volts power supply 1 is connected to a throw-over switch 2 by a potentiometer 3. The throw-over switch 2 is connected, on the one hand, to earth through a resistor 4 or read resistor (10Ω) and a voltmeter 5, as well as to the input of a voltage-current curve tracer 6 and, on the other hand, to sample 7 to be tested through a resistor 8 (50KΩ). The other terminal of sample 7 is connected to earth by a resistor 9 and a conductor 10 connects the other input of tracer 6 to one of the terminals of resistor 8.

FIG. 2 shows a detail of the assembly or sample 7.

Two cylindrical graphite pellets, numbered 11 and 12, and between which is disposed a pellet 13 of the sample of the product to be tested, are inserted between the conductors adapted to connect sample 7 to resistors 8 and 9 respectively (FIG. 1). Pellet 13 is maintained between the graphite cylinders by a conductive coating such as a silver paint put on the market by the German firm DEGUSSA. Pellet 13 is about 0.1 mm in thickness.

FIG. 3 is the voltage-current curve recorded with the device for sample 13 containing compound  $\text{Ca}_2\text{Na}_2\text{Al V}_3\text{O}_{12}$  (II). The voltages are shown in abscissa (volts) and the current in ordinates (milliamperes)

The graph shows that compound (II) has two states: 1. a resistive state corresponding to values

$$V = 140 \text{ V}, I = 0.12 \text{ m A} \text{ or } R \approx 1.17 \times 10^6 \Omega$$

2. a conductive state corresponding to the values

$$V = 5.5 \text{ V}$$

$$I = 4 \text{ m A} \text{ or } R \approx 1.37 \times 10^3 \Omega$$

On the curve, portion (A) corresponds to the resistive state and portion (B) to the reducer state.

## EXAMPLE 2

To obtain the product  $\text{Ca}_{1.86}\text{Na}_{2.14}\text{Al V}_3\text{O}_{11.86}\text{F}_{0.14}$  (I) (formula (I)  $x = 0.14 y = 0 z = 0$ )

The following mixture of oxides and carbonates, in which sodium fluoride is incorporated in the amounts given, are subjected to the same thermal treatment as described in example 1.

|                                   |           |
|-----------------------------------|-----------|
| 1.86 mole $\text{Ca CO}_3$        | 186.167 g |
| 1.0 mole $\text{Na}_2\text{CO}_3$ | 106.00 g  |
| 0.5 mole $\text{Al}_2\text{O}_3$  | 50.97 g   |
| 1.5 mole $\text{V}_2\text{O}_5$   | 363.80 g  |
| 0.14 mole $\text{NaF}$            | 5.88 g    |
| Total weight                      | 712.817 g |

A glass having a molecular weight of 586.977 g is obtained.

Formation of glass will not occur with fluoride ion contents higher than 0.14.

## EXAMPLE 3

To obtain the product  $\text{Ca}_2\text{Na}_2\text{Fe V}_3\text{O}_{12}$  (formula (I)  $x = 0 y = 1 z = 0$ ) as well as the product  $\text{Ca}_{2.4}\text{Na}_{2.4}\text{Al}_{0.2}\text{Fe V}_{3.6}\text{O}_{14.4}$ . This latter product, which does not correspond to the stoichiometric composition given in formula (I) can be obtained from the basic compound  $\text{Ca}_2\text{Na}_2\text{Al V}_3\text{O}_{12}$  (II) and from the compound  $\text{Ca}_2\text{Na}_2\text{Fe V}_3\text{O}_{12}$ .3a. The mixture corresponds to the compound  $\text{Ca}_2\text{Na}_2\text{Fe V}_3\text{O}_{12}$ 

|                                                     |          |
|-----------------------------------------------------|----------|
| 0.5 mole $\text{Fe}_2\text{O}_3$<br>and comprises : | 79.85 g  |
| 2.0 moles $\text{CaCO}_3$                           | 200.00 g |
| 1.0 mole $\text{Na}_2\text{CO}_3$                   | 106.00 g |
| 0.5 mole $\text{V}_2\text{O}_5$                     | 272.00 g |
| Total :                                             | 657.85 g |

This mixture is heated in a platinum crucible open to the air at 650°C for 2 hours then at 800°C for 2 hours. A reaction product is obtained which is ground fine.

3b. The product (3a) is mixed with 20 moles of product (II) also finely ground. The entire mixture is heated at 1,350°C for 6 hours in a covered platinum crucible. The glass forms on cooling.

## EXAMPLE 4

This example illustrates another variant of the vitreous composition which can be obtained from the products of examples 2 and (3b).

40 This product corresponds to the global formula :  $\text{Ca}_{2.34}\text{Na}_{2.42}\text{Al}_{1.04}\text{Fe}_{0.2}\text{V}_{3.72}\text{O}_{14.81}\text{F}_{0.14}$  A 0.2 mole (105.17g) mass of the product of example 3b is ground and mixed with 1 mole (586.977g) of the glass of example 2, which is also ground.

45 Said mixture is heated at 1,350°C for 6 hours in a covered platinum crucible. The glass forms on cooling.

## EXAMPLE 5

To obtain the product  $\text{Ca}_{2.4}\text{Y}_{0.2}\text{Na}_{2.4}\text{V}_{3.6}\text{O}_{14.4}$ 

This example illustrates a variant of the vitreous composition which can be obtained by mixing a compound containing yttrium and the basic product of example 1.

The following mixture is first prepared :

|                                   |          |
|-----------------------------------|----------|
| 0.5 mole $\text{Y}_2\text{O}_3$   | 112.92 g |
| 2.0 moles $\text{CaCO}_3$         | 200.00 g |
| 1.0 mole $\text{Na}_2\text{CO}_3$ | 106.00 g |
| 1.5 moles $\text{V}_2\text{O}_5$  | 272.00 g |

This mixture is heated at 650°C for 2 hours and at 800°C for 2 hours.

The resulting product is ground. An amount of 0.2 mole (138.18 g) of this finely ground compound is added to 1 mole (588.95 g) of the glass of example 1, which is also ground.

65 After mixing the product is heated for 6 hours at 1,350°C.

The glass forms on cooling.

## EXAMPLE 6 to 24

The following table gives details of a series of glass compositions which can be obtained according to the procedure described in example 1. In the first three col-

umns of the table the values of indices  $x$ ,  $y$  and  $z$ , corresponding to formula (I) are given. The glass formula is given in the fourth column and the amounts in moles and grams of the precursor products used are given in the last column, with their designation.

TABLE

| Ex | x    | y | z | Formula                                                                        | Precursor compounds (amounts in moles and in g)                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                            |
|----|------|---|---|--------------------------------------------------------------------------------|--------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 6  | 0.04 | 0 | 0 | $\text{Ca}_{1.96}\text{Na}_{2.04}\text{Al V}_3\text{O}_{11.96}\text{F}_{0.04}$ | 1.96, $\text{CO}_3\text{Ca}$ , 196.17 g.<br>1.00, $\text{CO}_3\text{Na}_2$ , 106 g.<br>1, $\text{Al}(\text{NO}_3)_3$ , 9 $\text{H}_2\text{O}$ , 375.14 g.<br>1.5, $\text{V}_2\text{O}_5$ , 272.65 g.<br>0.04, $\text{NaF}$ , 1.6788 g.<br>2, $\text{CO}_3\text{Ca}$ , 260.18 g.<br>1, $\text{CO}_3\text{Na}_2$ , 106 g.<br>0.9, $\text{Al}(\text{NO}_3)_3$ , 9 $\text{H}_2\text{O}$ , 337.62 g.<br>0.05, $\text{Fe}_2\text{O}_3$ , 7.979 g.<br>1.5, $\text{V}_2\text{O}_5$ , 272.85 g.<br>1.88, $\text{CO}_3\text{Ca}$ , 188.16 g.<br>1.00, $\text{CO}_3\text{Na}_2$ , 106 g.<br>0.90, $\text{Al}(\text{NO}_3)_3$ , 9 $\text{H}_2\text{O}$ , 337.62 g.<br>0.05, $\text{Fe}_2\text{O}_3$ , 7.979 g.<br>1.5, $\text{V}_2\text{O}_5$ , 272.85 g.<br>0.12, $\text{NaF}$ , 5.036 g.<br>2, $\text{CO}_3\text{Ca}$ , 200.18 g.<br>1, $\text{CO}_3\text{Na}_2$ , 106 g.<br>0.62, $\text{Al}(\text{NO}_3)_3$ , 9 $\text{H}_2\text{O}$ , 232.58 g.<br>0.19, $\text{Fe}_2\text{O}_3$ , 3.032 g.<br>1.5, $\text{V}_2\text{O}_5$ , 272.85 g.<br>1.88, $\text{CO}_3\text{Ca}$ , 188.16 g.<br>1.00, $\text{CO}_3\text{Na}_2$ , 106 g.<br>0.62, $\text{Al}(\text{NO}_3)_3$ , 9 $\text{H}_2\text{O}$ , 232.58 g.<br>0.19, $\text{Fe}_2\text{O}_3$ , 3.032 g.<br>1.5, $\text{V}_2\text{O}_5$ , 272.85 g.<br>0.12, $\text{NaF}$ , 5.036 g.<br>1.80, $\text{CO}_3\text{Ca}$ , 180.16 g.<br>0.05, $\text{La}_2\text{O}_3$ , 16.29 g.<br>0.05, $\text{Y}_2\text{O}_3$ , 11.30 g.<br>1.05, $\text{CO}_3\text{Na}_2$ , 111.30 g.<br>1.0, $\text{Al}(\text{NO}_3)_3$ , 9 $\text{H}_2\text{O}$ , 375.14 g.<br>1.5, $\text{V}_2\text{O}_5$ , 272.85 g.<br>1.66, $\text{CO}_3\text{Ca}$ , 166.14 g.<br>0.05, $\text{La}_2\text{O}_3$ ou $\text{Y}_2\text{O}_3$   $\text{La}_2\text{O}_3$ , 16.29 g.<br>$\text{Y}_2\text{O}_3$ , 11.29 g.<br>1.05, $\text{CO}_3\text{Na}_2$ , 111.30 g.<br>1.00, $\text{Al}(\text{NO}_3)_3$ , 9 $\text{H}_2\text{O}$ , 375.14 g.<br>1.5, $\text{V}_2\text{O}_5$ , 272.85 g.<br>0.14, $\text{FNa}$ , 5.87 g.<br>1.8, $\text{CO}_3\text{Ca}$ , 180.16 g.<br>0.05, $\text{La}_2\text{O}_3$ ou $\text{Y}_2\text{O}_3$   $\text{La}_2\text{O}_3$ , 16.29 g.<br>$\text{Y}_2\text{O}_3$ , 11.29 g.<br>1.05, $\text{CO}_3\text{Na}_2$ , 111.30 g.<br>0.90, $\text{Al}(\text{NO}_3)_3$ , 9 $\text{H}_2\text{O}$ , 337.62 g.<br>0.05, $\text{Fe}_2\text{O}_3$ , 7.97 g.<br>1.5, $\text{V}_2\text{O}_5$ , 272.85 g.<br>1.68, $\text{CO}_3\text{Ca}$ , 168.15 g.<br>0.05, $\text{La}_2\text{O}_3$ ou $\text{Y}_2\text{O}_3$   $\text{La}_2\text{O}_3$ , 16.29 g.<br>$\text{Y}_2\text{O}_3$ , 11.29 g.<br>1.05, $\text{CO}_3\text{Na}_2$ , 111.30 g.<br>0.9, $\text{Al}(\text{NO}_3)_3$ , 9 $\text{H}_2\text{O}$ , 337.62 g.<br>0.05, $\text{Fe}_2\text{O}_3$ , 7.97 g.<br>1.5, $\text{V}_2\text{O}_5$ , 272.85 g.<br>0.12, $\text{FNa}$ , 5.036 g.<br>1.66, $\text{CO}_3\text{Ca}$ , 166.14 g.<br>0.05, $\text{La}_2\text{O}_3$ ou $\text{Y}_2\text{O}_3$   $\text{La}_2\text{O}_3$ , 16.29 g.<br>$\text{Y}_2\text{O}_3$ , 11.29 g.<br>1.05, $\text{CO}_3\text{Na}_2$ , 111.30 g.<br>0.8, $\text{Al}(\text{NO}_3)_3$ , 9 $\text{H}_2\text{O}$ , 300.11 g.<br>1.5, $\text{V}_2\text{O}_5$ , 272.85 g.<br>0.1, $\text{Fe}_2\text{O}_3$ , 15.95 g.<br>1.68, $\text{CO}_3\text{Ca}$ , 168.15 g.<br>0.05, $\text{La}_2\text{O}_3$ ou $\text{Y}_2\text{O}_3$   $\text{La}_2\text{O}_3$ , 16.29 g.<br>$\text{Y}_2\text{O}_3$ , 11.29 g.<br>1.05, $\text{CO}_3\text{Na}_2$ , 117.66 g.<br>0.8, $\text{Al}(\text{NO}_3)_3$ , 9 $\text{H}_2\text{O}$ , 300.11 g.<br>0.1, $\text{Fe}_2\text{O}_3$ , 15.95 g.<br>1.5, $\text{V}_2\text{O}_5$ , 272.85 g.<br>0.12, $\text{FNa}$ , 5.036 g.<br>1.4, $\text{CO}_3\text{Ca}$ , 140.12 g.<br>0.1, $\text{La}_2\text{O}_3$ ou $\text{Y}_2\text{O}_3$   $\text{La}_2\text{O}_3$ , 16.29 g.<br>$\text{Y}_2\text{O}_3$ , 11.29 g.<br>1.1, $\text{CO}_3\text{Na}_2$ , 116.6 g.<br>0.8, $\text{Al}(\text{NO}_3)_3$ , 9 $\text{H}_2\text{O}$ , 300.11 g.<br>0.1, $\text{Fe}_2\text{O}_3$ , 15.95 g.<br>1.5, $\text{V}_2\text{O}_5$ , 272.85 g.<br>1.48, $\text{CO}_3\text{Ca}$ , 148.13 g.<br>0.10, $\text{Y}_2\text{O}_3$ ou $\text{La}_2\text{O}_3$   $\text{La}_2\text{O}_3$ , 16.29 g.<br>$\text{Y}_2\text{O}_3$ , 11.29 g.<br>1.10, $\text{CO}_3\text{Na}_2$ , 116.6 g.<br>0.8, $\text{Al}(\text{NO}_3)_3$ , 9 $\text{H}_2\text{O}$ , 300.11 g.<br>0.1, $\text{Fe}_2\text{O}_3$ , 15.95 g.<br>1.5, $\text{V}_2\text{O}_5$ , 272.85 g.<br>0.12, $\text{FNa}$ , 5.036 g. |

TABLE—Continued

| Ex | x    | y    | z    | Formula                                                           | Precursor compounds (amounts in moles and in g)                                                                                                                                                                                                                                   |
|----|------|------|------|-------------------------------------------------------------------|-----------------------------------------------------------------------------------------------------------------------------------------------------------------------------------------------------------------------------------------------------------------------------------|
| 19 | 0    | 0    | 0.24 | $Ca_{1.52}Ln_{0.24}Na_{2.24}Al_1V_3O_{12}$                        | 1.52, $CO_3Ca$ , 152.13 g.<br>0.12, $Y_2O_3$ ou $La_2O_3$ $  La_2O_3$ , 16.29 g.<br>$  Y_2O_3$ , 11.29 g.<br>1.12, $CO_3Na_2$ , 118.72 g.<br>1, $Al(NO_3)_3$ , 9H <sub>2</sub> O, 375.14 g.<br>1.5, $V_2O_5$ , 272.85 g.                                                          |
| 20 | 0.12 | 0    | 0.24 | $Ca_{1.40}Ln_{0.24}Na_{2.36}Al_1V_3O_{11.88}F_{0.12}$             | 1.40, $CO_3Ca$ , 140.12 g.<br>0.12, $La_2O_3$ ou $Y_2O_3$ $  La_2O_3$ , 16.29 g.<br>$  Y_2O_3$ , 11.29 g.<br>1.12, $CO_3Na_2$ , 118.72 g.<br>1.0, $Al(NO_3)_3$ , 9H <sub>2</sub> O, 375.14 g.<br>0.12, $FNa$ , 5.036 g.<br>1.5, $V_2O_5$ , 272.85 g.                              |
| 21 | 0    | 0.10 | 0.24 | $Ca_{1.52}Ln_{0.24}Na_{2.24}Al_{0.90}Fe_{0.10}V_3O_{12}$          | 1.52, $CO_3Ca$ , 152.13 g.<br>0.12, $La_2O_3$ ou $Y_2O_3$ $  La_2O_3$ , 16.29 g.<br>$  Y_2O_3$ , 11.29 g.<br>1.12, $CO_3Na_2$ , 118.72 g.<br>0.90, $Al(NO_3)_3$ , 9H <sub>2</sub> O, 337.62 g.<br>0.05, $Fe_2O_3$ , 7.97 g.<br>1.5, $V_2O_5$ , 272.85 g.                          |
| 22 | 0.12 | 0.10 | 0.24 | $Ca_{1.40}Ln_{0.24}Na_{2.36}Al_{0.9}Fe_{0.1}V_3O_{11.88}F_{0.12}$ | 1.40, $CO_3Ca$ , 140.12 g.<br>0.12, $La_2O_3$ ou $Y_2O_3$ $  La_2O_3$ , 16.29 g.<br>$  Y_2O_3$ , 11.29 g.<br>1.12, $CO_3Na_2$ , 118.72 g.<br>0.9, $Al(NO_3)_3$ , 9H <sub>2</sub> O, 337.62 g.<br>0.05, $Fe_2O_3$ , 7.97 g.<br>1.5, $V_2O_5$ , 272.85 g.                           |
| 23 | 0    | 0.20 | 0.24 | $Ca_{1.52}Ln_{0.24}Na_{2.24}Al_{0.8}Fe_{0.2}V_3O_{12}$            | 1.52, $CO_3Ca$ , 152.13 g.<br>0.12, $La_2O_3$ ou $Y_2O_3$ $  La_2O_3$ , 16.29 g.<br>$  Y_2O_3$ , 11.29 g.<br>1.12, $CO_3Na_2$ , 118.72 g.<br>0.8, $Al(NO_3)_3$ , 9H <sub>2</sub> O, 300.11 g.<br>0.2, $Fe_2O_3$ , 15.95 g.<br>1.5, $V_2O_5$ , 272.85                              |
| 24 | 0.12 | 0.20 | 0.24 | $Ca_{1.40}Ln_{0.24}Na_{2.36}Al_{0.8}Fe_{0.12}V_3O_{11.88}$        | 1.40, $CO_3Ca$ , 140.12 g.<br>0.12, $La_2O_3$ ou $Y_2O_3$ $  La_2O_3$ , 16.29 g.<br>$  Y_2O_3$ , 11.29 g.<br>1.12, $CO_3Na_2$ , 118.72 g.<br>0.8, $Al(NO_3)_3$ , 9H <sub>2</sub> O, 300.11 g.<br>0.1, $Fe_2O_3$ , 15.95 g.<br>1.5, $V_2O_5$ , 181.90 g.<br>0.12, $FNa$ , 5.036 g. |

The invention is naturally not limited to the above examples which are essentially illustrative and describe a certain number of specific vitreous compounds corresponding to the requirements of the invention and having bistable electrical characteristics.

We claim:

1. A vitreous compound with bistable electrical characteristics corresponding to formula (I)



wherein the letters have the usual meaning of the elements in the Periodic Table, with the exception of Ln which designates an element which is a part of the group of rare earths belonging to the class of lanthanides and yttrium, whereas x, y and z each represent numbers in the range of 0 to 1, which are bound together by ionic equilibrium relationships.

2. The compound of claim 1 wherein x is zero.  
3. The compound of claim 1 wherein y is zero.  
4. The compound of claim 1 wherein z is zero.  
5. The compound of claim 1 wherein x, y and z are simultaneously zero, the said compound corresponding to the formula :



6. The compound of claim 1, wherein the element Ln is lanthanum and z is greater than 0.  
7. The compound of claim 1 wherein x, y and z comply with the inequalities

$$x < 0.15$$

$$y < 0.5$$

and

$$z < 0.3$$

40 8. A process for the production of a compound of formula (I):



45 wherein the letters have the usual meanings of the elements in the Periodic Table with the exception of Ln which designates an element which is a part of the group of rare earths belonging to the class of lanthanides and yttrium, whereas x, y and z each represent

50 numbers in the range of 0 to 1, which are bound together by ionic equilibrium relationships, said process comprising the steps, (a) preparation of an intimate mixture of precursor products containing the elements of said compound in substantially stoichiometric proportions, (b) heating said mixture at a temperature higher than about 1,300°C for at least 5 hours and, (c) cooling of said heated mixture to normal temperature, the desired vitreous compound forming during said cooling.

55 9. The process of claim 8, wherein the heating (b) is carried out for about 6 to 12 hours.

10. The process of claim 8, wherein during the heating (b) the temperature is maintained between about 1,300° and 1,400°C.